

# UNITED STATES PATENT OFFICE.

ELBRIDGE W. STEVENS, OF BALTIMORE, MARYLAND, ASSIGNOR TO CHEMICAL FUEL COMPANY OF AMERICA, INC., OF LOUISVILLE, KENTUCKY, A CORPORATION OF DELAWARE.

## MOTOR FUEL.

1,414,759.

Specification of Letters Patent. Patented May 2, 1922.

No Drawing.

Application filed March 9, 1920. Serial No. 364,386.

To all whom it may concern:

Be it known that I, ELBRIDGE WEBSTER STEVENS, a citizen of the United States, residing at Baltimore, in the State of 5 Maryland, have invented certain new and useful Improvements in Motor Fuels, of which the following is a specification.

This invention relates to motor fuels; and it comprises a composite motor fuel consisting of a hydrocarbon oil, such as kerosene (or other petroleum oil) and alcohol (together with a hydrocarbon blending agent if necessary,) and in addition containing a small amount of a readily volatile 15 ester of formic acid, such as methyl formate or ethyl formate; all as more fully herein-after set forth and as claimed.

In the manufacture of many composite motor fuels by methods now in use, or proposed, the bulk of the composition is made 20 of alcohol and a petroleum or coal tar hydrocarbon oil. Kerosene and even heavier oils, such as gas oil or solar oil, are used. Or specially made distillates may 25 be used. Usually a blending agent, such as benzol, is used to promote miscibility of the oil and alcohol and make the composition stable. For this purpose any co-solvent can be used; that is a body capable 30 of dissolving both the alcohol and the oil, or of dissolving in both.

With most of these compositions it is desirable to use a modicum of some rather volatile combustible body to give quicker 35 ignition in the engine. The petroleum oils ordinarily employed in these mixtures are not very volatile and the alcohol is not as readily volatile as is desirable for engine purposes. As this quick-ignition material 40 various esters of acetic acid, such as ethyl acetate, methyl acetate, butyl acetate, etc., made by combining acetic acid with the corresponding alcohol have been proposed and used, as they are highly volatile, 45 readily combustible bodies. Valerates, buty- 50 rates, etc., have also been proposed. The use of these materials is, however, subject to the objection that in the engine cylinder they tend to decompose more or less with the re-formation of the original alcohol and of the acid from which they were made; re-forming acetic acid in the case of ethyl or methyl acetate. The amount of this acid is not large, but it is sufficient to produce 55 more or less corrosion of metal parts con-

tacting with the explosion gases to obviate the effects of this acidity it has been proposed in the prior art to incorporate a basic body capable of neutralizing the 60 acidity developed.

In the present invention in lieu of using these esters I employ the corresponding esters of formic acid which, unlike the acetates, butyrates, valerates, etc., do not break up with formation of free acids 65 since acidity does not develop the use of basic bodies is unnecessary. The formate esters are even more volatile than the acetate esters, so that smaller quantity suffices to give quick ignition to the fuel; and they 70 are also held back better by the composition. Acetic acid esters tend to evaporate away from oil-alcohol compositions in time; this tendency being greater than with the formates. Ethyl formate, methyl formate 75 or butyl formate may be used for the present purposes.

Formic acid has the empirical composition of  $\text{CH}_2\text{O}_2$  and when heated it breaks up readily into  $\text{H}_2\text{O}$  and  $\text{CO}$ ; neither of 80 which is acid. Similarly, ethyl formate and methyl formate on heating yield the corresponding alcohols and  $\text{CO}$ . Both are therefore harmless in the engine.

Ethyl formate may be readily made by 85 distilling ethyl alcohol with sodium formate in the presence of an acid, such as hydrochloric acid or sulfuric acid. The sodium formate is readily obtained commercially and is a cheap material made by absorbing 90 the carbon monoxide of producer gas with caustic soda. Methyl formate may be made from sodium formate and methyl alcohol in the presence of an acid. Ethyl formate boils at 55° C. or 131° F. and has a high 95 vapor tension at ordinary temperatures. Methyl formate is still more volatile, boiling at about 30° C. or 86° F.

While I have described the use of the formate esters more particularly with regard to the composite fuels made up of admixed hydrocarbon oils and alcohols, it is obvious that they may be used with either alone or in admixture with any motor fuel to which it is desired to give a quicker ignition.

It is not ordinarily necessary or desirable to use more than a very small quantity of formate esters; say not more than about 5 per cent on the weight of the total com-

60

75

80

95

100

105

110

position. For some purposes, as in making aviation fuel the amount may be somewhat increased; but ordinarily the amount mentioned will suffice.

5 A typical composition under the present invention can be made by blending say, 75 parts of a suitable petroleum distillate with about 15 parts of alcohol, using about 5 parts of toluol as a co-solvent or blending 10 agent. To this mixture may be added about 5 parts of ethyl formate or methyl formate. The petroleum distillate used may be ordinary kerosene, gas oil, cracked distillate,

etc., or various petroleum distillates may be blended. The composition will tolerate a 15 considerable proportion of rather heavy distillate.

What I claim is:—

A motor fuel of the same general character as gasoline consisting of a petroleum distillate, alcohol, a hydrocarbon blending agent and a small amount of a readily volatile formic acid ester. 20

In testimony whereof, I affix my signature.

ELBRIDGE W. STEVENS